

1

2,758,086

## LUBRICANT COMPOSITION

Frank A. Stuart, Richmond, and Warren Lowe, Berkeley, Calif., assignors to California Research Corporation, San Francisco, Calif., a corporation of Delaware

No Drawing. Application June 28, 1952,  
Serial No. 296,248

9 Claims. (Cl. 252—32.5)

This invention relates to a lubricant composition, and is particularly directed to the provision of a composition of their character which incorporates a branched chain amino compound.

It is known that amines and amine salts have the ability to impart good detergency characteristics to lubricating oils, whereby the various insoluble products formed as a result of oxidative attack on the fuel or from combustion of the fuel are maintained in suspension in the oil. However, while the amino compounds which have heretofore been employed in lubricating oils possess satisfactory detergency qualities, their field of application as lubricant additives has been greatly curtailed due to their unfavorable action from a corrosion standpoint under the more rigorous conditions of service. Thus, while oils containing amino additives are satisfactory and do not appear to have any adverse effects when employed under mild service conditions, such oils are not adapted for use in Diesel and other internal combustion engines which are operated at relatively elevated temperatures. Corrosion difficulties with amine-compounded oils soon become severe in such service, particularly in the presence of metals which are susceptible to attack by acidic and/or peroxidic decomposition products of the oil or other materials. Bearing metals such as copper-lead, cadmium-silver, cadmium-nickel, so-called high lead bearing alloys, and the like, are particularly prone to attack by these decomposition products, and it appears that under the more rigorous operating conditions mentioned above, the amino compounds actually promote corrosion of the bearing metal surfaces by the oil.

As is pointed out in copending application, Serial No. 237,684, filed July 19, 1951, many of the oil additives which normally act to suppress or inhibit this corrosive attack on bearing metal surfaces are not appreciably effective for this purpose when employed in oils containing amino additives, particularly when said oils are employed in Diesel and other internal combustion engines where relatively high temperature conditions are encountered. It is disclosed in said copending application that oxidation attack on hard bearing metals at elevated temperatures by amino compound-containing oils can be reduced to the desired minimum by the addition to the oil of a benzothiazyl dialiphatic dithiocarbamate. However, while use of the latter inhibitors is satisfactory from a performance standpoint, they are relatively expensive chemicals, and the introduction thereof into the oil materially adds to the cost of the product.

Accordingly, it would be desirable if a class of amino compounds were available which would impart good detergency characteristics to lubricating oils without appreciably increasing the corrosivity of the resulting composition to bearing metal surfaces even under rigorous service conditions, and it forms the principal object of this invention to provide such a class of amino compounds. It is our discovery that by incorporating in an oil of lubricating viscosity a minor percentage of one or more amines or amine salts of the type having at least one

2

branched aliphatic chain of 10 or more carbon atoms attached to the amino nitrogen atom, there is obtained a composition having excellent detergency characteristics and low corrosivity to bearing metal and other surfaces coming into contact with the oil under all service conditions. These beneficial results are obtained without the necessary use in the oil of dithiocarbamate or other corrosion-inhibitory additives. Further, it has been found that the branched chain amino compounds disclosed herein are superior to other amino compounds in that they are more resistant to oxidative attack and have a lower pour point.

More specifically, the amino compounds which are useful in a practice of the present invention are those of the type having the general formula



In the formula R<sub>1</sub> is a branched chain radical of aliphatic character containing at least 10 carbon atoms, which terminology is employed herein to designate both unsubstituted aliphatic radicals, as well as those which are substituted to a minor extent by one or more substituent groups such as phenyl, benzyl, cyclohexyl, chloro, amino, hydroxy, or the like. R<sub>2</sub> and R<sub>3</sub> in said formula are selected from the group consisting of hydrogen atoms and organic radicals which are essentially hydrocarbonaceous in character. By essentially hydrocarbonaceous radicals are meant those which are composed mainly of hydrogen and carbon, but which can also contain minor amounts of non-hydrocarbon substituents such as chloro, bromo, hydroxyl and amino groups.

In the preferred practice of this invention R<sub>1</sub> represents a branched chain alkyl group of 10 or more carbon atoms which, more preferably, is attached to the amino nitrogen atom through a tertiary carbon atom, while R<sub>2</sub> and R<sub>3</sub> are preferably hydrogen atoms or hydrocarbon radicals.

The following primary, secondary and tertiary amines are illustrative of those which can be employed in carrying out the present invention:

### PRIMARY AMINES

45 "Isooctadecyl" amine<sup>1</sup>  
1,1-dimethyldodecylamine  
1,1-dimethyloctadecylamine  
50 1-methyl-1-benzyl-tridecylamine  
1-methyl-1-isopropyloctylamine  
1,1-diethyl-4-methyldodecylamine  
1,1,4,6,6-pentamethylheptylamine  
1,1,3,3,5,5-hexamethylhexylamine  
1-methyl-4-ethyloctylamine  
55 1-(3-ethylpentyl)-4-ethyloctylamine  
1-sec.butyl-4-ethyloctylamine  
2-ethyloctylamine  
1-phenyl-2,2-dimethyldecylamine  
1-methyl-4-ethylheptadecylamine  
60 1-benzyl-2-methyldodecylamine  
2-isopropyl-nonylamine  
9-methyldecylamine  
1-methyl-4-propyl-10-aminodecylamine  
2-isopropyl-6-hydroxydodecylamine

### SECONDARY AMINES

N-amyl-1-methyl-4-ethyloctylamine  
di-(1-methyldodecyl)amine  
N-butyl-“isooctadecyl” amine  
N-n-octadecyl-“isooctadecyl” amine  
N-phenyl-2-isopropyldecylamine  
N-cyclohexyl-1-methyl-3-ethylheptadecylamine

N-benzyl-2-ethyldecylamine  
N-methallyl-1-sec. butyloctylamine  
N-methyl-2-ethyl-4-decylamine

## TERTIARY AMINES

N,N-dimethyl-1-sec. butyl-4-ethyloctylamine  
N-ethyl-N-butyl-1-methyl-4-ethyloctylamine  
N-methyl-N-phenyl-1,1-dimethyldodecylamine

<sup>1</sup> The product "isoctadecylamine" is marketed by Rohm and Haas Company under the trade name "Primene JM-R," the "isoctadecyl" radical in this compound being derived from the polymerization of isobutylene. The formula of this product, wherein the amino nitrogen atom is attached directly to a tertiary carbon atom, is mainly  $C_{18}H_{37}NH_2$  to  $C_{20}H_{41}NH_2$ . It has a specific gravity (25° C.) of 0.828, a refractive index (25° C.) of 1.455, and a boiling point range (5 to 95%) of from 275 to 340° C. at 760 mm./Hg. Other "isoctadecylamines" mentioned herein are obtained by replacement of one or both of the hydrogen atoms on the amine nitrogen atom by the indicated radical(s).

The amine salts whose use comes within the scope of the present invention are those of the type which can be formed by reacting the above or other suitable branched chain amines with various inorganic or organic acids, including mono- or poly-basic carboxylic acids, as well as sulfonic or phosphonic acids. Representative acids which can be employed in forming the branched chain amine salts are formic, acetic, propionic, butyric, caproic, lauric, stearic, arachidic, oleic, benzoic, toluic, naphthenic, cetylphosphoric, cyclohexanephosphonic, cetylulfuric, petroleum sulfonic, maleic, tartic, benzoic, phthalic, citric, chlorostearic, phenylstearic and mercaptostearic acids. In forming the salts, the polybasic acids can either be used as such or as the partial esters with various alcohols such as ethanol, hexanol, hexadecanol and the like. Representative branched chain amine salts are "isoctadecyl" amine benzoate, di(1-methyl-4-ethyldodecylamine) adipate, 1-isopropyldecylamino oleate, N,N-dimethyl-1-sec. butyloctylamine naphthenate, 1-(3-ethylpentyl) - 4 - ethyloctylamine acetate, N-amyl-1-methyl-4-ethyldecylamine cyclohexanephosphonate, 1 - methyl - 4 - ethyldecylamine cetylulfate and 2-isopropyldecylamine phenylmaleate.

The branched chain amine and amine salts of the present invention effect the desired improvement in the base oil when added thereto in minor percentages, and good results have been obtained using from about 1 to 20% by weight of the amine or amine salt additive. In some cases amounts considerably smaller than 1%, as from about 0.1 to 0.3%, impart appreciable detergent properties to the oil, and amounts as small as this can frequently be employed, particularly when the oil is also fortified with other additives. Conversely, amounts of the present additive larger than 20% can be employed on occasion, as for example when the oil is to be used in engines known to generate exceptionally large quantities of acids on combustion of their fuels, and again in lubricants which are compounded with exceptionally large quantities of the additive and are primarily intended to be combined with more dilute, or uncompounded lubricant oils.

The compounding agents of this invention are not limited in their applicability to any particular base oil stock, but can be combined with any oil having the desired lubricating properties. Thus, depending on the conditions and service which the compounded oil is to encounter, the base oil stock can be a Pennsylvania or other paraffinic base oil, a refined naphthenic base oil, or a synthetic hydrocarbon or non-hydrocarbon oil of lubricating viscosity. As synthetic oils there can be mentioned alkylated waxes and other hydrocarbons of high molecular weight, hydrogenated polymers of olefin hydrocarbons and the condensates of chlorinated alkyl hydrocarbons with aryl compounds. Other suitable synthetic oils are those which are obtained by the polymerization of lower molecular weight alkylene oxides such as propylene and/or ethylene oxide. Still other synthetic oils are obtained by etherification and/or

esterification of the hydroxy groups in alkylene oxide polymer such as, for example, the acetate of the 2-ethylhexanol-initiated polymer of propylene oxide. Another important class of synthetic oils comprises the high molecular weight esters, as, for example, di(ethylhexyl) sebacate.

The compounded oils of this invention find utility not only as crankcase lubricants for internal combustion engines (including spark-ignition and diesel engines), but also as turbine oils, cable oils, electric switch oils, transformer oils and hydraulic oils and the like. Further, the branched chain amino compounding agents of this invention can be added to the base oil in conjunction with other additives such as other mineral oil detergents (e. g., polyvalent metal phenates, sulfonates, thiophosphates, etc.), pour point depressants, oiliness agents, extreme pressure addition agents, anti-oxidants, corrosion-inhibiting agents, blooming agents, compounds for enhancing the viscosity index of the oil, and thickening agents. There also can be employed metal soaps in either grease-forming proportions or in amounts insufficient to form grease, as in the case of mineral castor machine oils or other compounded liquid lubricants. In many cases, it is desirable to avoid the use of metal-containing additives, in which case only secondary ingredients of non-metallic character should be added to the oil.

The following examples illustrate the present invention in various of its embodiments.

## Example I

In this operation the corrosivity of a lubricant composition containing branched chain amine or amine salt additives was measured and compared with that of the un compounded base oil as well as with that of the same base oil compounded with a non-branched chain amine or amine salt additive. In these tests the base oil employed was a highly refined product of SAE 30 grade having a V. I. of 85 and derived from California waxy crude. These tests were conducted by immersing highly polished sections of a copper-lead bearing insert measuring about  $2\frac{1}{2}'' \times 3\frac{1}{8}'' \times 1''$  of known weight in the test oil. The oil surrounding the insert was then heated to a temperature of 300° F. and maintained at this temperature, with stirring, for 20 hours. At the end of this time the strip was removed from the oil and cleaned, first with chloroform and then with petroleum ether. The cleaned strip was then weighed and the difference in weight between the original strip and the solvent-washed strip was noted and recorded as weight loss due to corrosion by the oil composition. Other tests were conducted in the same manner, but with the specimen being left in the heated test oil, with stirring, for a period of 40 hours. In each case the additive was present in the amount of 5%, except in the case of the base oil, which contained no additive. The weight loss experienced by the test specimens in the various oil compositions is given in Table I below.

TABLE I  
[Cu-Pb strip corrosion data]

|    | Additive                             | Weight Loss (mgs.) |         |
|----|--------------------------------------|--------------------|---------|
|    |                                      | 20 Hrs.            | 40 Hrs. |
| 65 | None                                 | 45.6               | 65.4    |
|    | Isooctadecylamine                    | 41.6               | 64.3    |
|    | N-butyl-isoctadecylamine             | 15.4               | 42.4    |
|    | N-octadecyl-isoctadecylamine         | 57.5               | 75.5    |
|    | N-dodecylamine                       | 289.4              | 441.3   |
|    | N-octadecylamine                     | 278.7              | 451.4   |
|    | di-n-octadecylamine                  | 146.2              | 171.1   |
|    | Isooctadecylamine alkaneephosphonate | 53.9               | 95.4    |
| 70 | n-octadecylamine alkanephosphonate   | 321.1              | 414.9   |
|    | Isooctadecylamine cetylmaleate       | 90.3               | 122.3   |
|    | n-dodecylamine cetylmaleate          | 169.5              | 261.9   |
|    | Isooctadecylamine oleate             | 105.6              | 133.5   |
|    | n-octadecylamine oleate              | 249.4              | 388.4   |

<sup>1</sup> The alkanephosphonate is derived from petroleum white oil.

From the above data, it will be seen that the lubricant compositions compounded with branched chain amines and amine salts afford a degree of protection from corrosion which is far superior to that of the other compounds tested, and oils which are relatively non-corrosive as shown by this test are admirably suited for use, not only in diesel and other internal combustion engines, but also as electrical insulating oils, cable oils, turbine oils and the like, as well.

*Example II*

In this operation the detergency qualities imparted to a base oil by the addition of 5% iso-octadecylamine are measured and compared with those of the uncompounded base oil (a highly refined base oil, SAE 30, 85 V. I., derived from California waxy crude), as well as with those of a commercial heavy duty oil (of the same base stock) now commonly employed in diesel engines. In this test a C. R. C., L-1 type Caterpillar single cylinder test engine was maintained in continuous operation for a period of 120 hours, the exhaust temperature being 800° F. The quality of the oil was evaluated at the end of the run by disassembling the engine and inspecting the four ring grooves in the piston for deposit and the intervening lands for discoloration. The amount of deposit found to be present in each groove is expressed in Table II below in terms of "G. D." (Groove Deposit) numbers, the scale employed being 0 to 100, with 0 indicating the absence of any deposit and with 100 indicating a complete filling of the groove. The extent of discoloration on the lands was measured and is expressed in Table II below in terms of Land "P. D." (Piston Discoloration) numbers. In obtaining the P. D. numbers, a value of 0 was assigned to a land which was completely clean, whereas one which was completely black was given a value of 800, with intermediate numbers being assigned to areas falling between these two extremes. The fuel employed contained between 0.4 and 1% sulfur.

TABLE II  
[L-1 type Caterpillar engine data (120 hrs.-800° F. exhaust temp.).]

| Lubricant                           | G. D. Nos. |        |        |        | Land P. D. Nos. |        |        |
|-------------------------------------|------------|--------|--------|--------|-----------------|--------|--------|
|                                     | Ring 1     | Ring 2 | Ring 3 | Ring 4 | Land 1          | Land 2 | Land 3 |
| Base Oil.....                       | 35         | 14     | 10     | 10     | 800             | 800    | 800    |
| Base Oil+5% iso-octadecylamine..... | 15         | 0      | 0      | 0      | 0               | 0      | 0      |
| Commercial Heavy Duty Oil.....      | 19         | 8      | 4      | 4      | 425             | 0      | 0      |

We claim:

1. A lubricant composition comprising a major portion of an oil of lubricating viscosity and a minor percentage, sufficient to impart detergent qualities to the oil, of at least one amino compound selected from the group consisting of (1) alkyl amines having attached to the amino nitrogen atom at least one branched chain alkyl radical having at least 10 carbon atoms, said alkyl radical being attached to the amino nitrogen atom through a tertiary carbon atom and (2) salts of said

amines and an organic acid selected from the group consisting of oleic acid, cetyl maleic acid and alkane phosphonic acid derived from petroleum white oil, said composition being characterized by low corrosivity to bearing and other metal surfaces.

2. The composition of claim 1, wherein the amino compound is present in an amount of from about 1 to 20% by weight.

3. A lubricant composition comprising a major portion of an oil of lubricating viscosity and a minor percentage, sufficient to impart detergent qualities to the oil, of an alkyl amine having attached to the amino nitrogen atom at least one branched chain alkyl radical having at least 10 carbon atoms, said alkyl radical being attached to the amino nitrogen atom through a tertiary carbon atom said composition being characterized by low corrosivity to bearing and other metal surfaces.

4. A lubricant composition comprising a major portion of an oil of lubricating viscosity and a minor percentage, sufficient to impart detergent qualities to the oil, of a salt of an alkyl amine and an organic acid selected from the group consisting of oleic acid, cetyl maleic acid and alkane phosphonic acid derived from petroleum white oil having attached to the amino nitrogen atom at

least one branched chain alkyl radical having at least 10 carbon atoms, said alkyl radical being attached to the amino nitrogen atom through a tertiary carbon atom, said composition being characterized by low corrosivity to bearing and other metal surfaces.

5. A lubricant composition comprising a major portion of an oil of lubricating viscosity and a minor percentage, sufficient to impart detergent qualities to the oil, of an alkyl amine wherein at least one alkyl radical containing at least 10 carbon atoms is attached to the amino nitrogen atom through a tertiary carbon atom, said composition being characterized by low corrosivity to bearing and other metal surfaces.

6. A lubricant composition comprising a major portion of an oil of lubricating viscosity and a minor percentage, sufficient to impart detergent qualities to the oil, of a salt of an alkyl amine and an organic acid selected from the group consisting of oleic acid, cetyl maleic acid and alkane phosphonic acid derived from petroleum white oil wherein at least one alkyl radical containing at least 10 carbon atoms is attached to the amino nitrogen atom through a tertiary carbon atom, said composition being characterized by low corrosivity to bearing and other metal surfaces.

7. The composition of claim 5, wherein the amine is iso-octadecyl amine.

8. The composition of claim 5, wherein the amine is N-butyl-iso-octadecyl amine.

9. The composition of claim 5, wherein the amine is N-n-octadecyl-iso-octadecyl amine.

References Cited in the file of this patent

UNITED STATES PATENTS

- |           |           |       |               |
|-----------|-----------|-------|---------------|
| 1,888,023 | Adams     | ----- | Nov. 15, 1932 |
| 2,234,096 | Teter     | ----- | Mar. 4, 1941  |
| 2,413,852 | Turner    | ----- | Jan. 7, 1947  |
| 2,476,271 | Bartleson | ----- | July 19, 1949 |